

1,108,243.

H. C. RYDING.

METHOD OF TREATING INGOTS.

APPLICATION FILED MAR. 31, 1913. RENEWED FEB. 12, 1914.

Patented Aug. 25, 1914.



Witnesses:

Harold G. Bennett  
Chas J. Murray

Inventor:  
Herbert C. Ryding  
By Lanthier & Bell, Attys.

# UNITED STATES PATENT OFFICE.

HERBERT C. RYDING, OF BIRMINGHAM, ALABAMA.

## METHOD OF TREATING INGOTS.

1,108,243.

Specification of Letters Patent. Patented Aug. 25, 1914.

Application filed March 31, 1913, Serial No. 757,987. Renewed February 12, 1914. Serial No. 818,388.

To all whom it may concern:

Be it known that I, HERBERT C. RYDING, a citizen of the United States, residing at Birmingham, in the county of Jefferson and State of Alabama, have invented certain new and useful Improvements in Methods of Treating Ingots, of which the following is a specification.

My invention relates to the art of metal rolling and has particular reference to a novel method of treating steel ingots prior to the reduction thereof by rolling.

During the past two or three years the subject of rail failures has persistently forced itself upon the attention of railway managers and rail manufacturers, with the result that searching investigations have been carried out in connection with the present methods of manufacture, and subsequent treatment of rails, the object of which was to determine if possible what were the real causes leading up to rail failures.

Segregating out from the mass of detail on this subject the chief causes of failure, it will be found that by far the greater number of failures proceed from one or two causes: First in importance I believe is seamy steel and, second, piped ingots.

Seams in rails either proceed from blow holes in the ingot or from the formation of cracks in the sides, commonly noted during the passage of the ingot through the first few passes in the blooming mill rolls. By far the greater number of these seams proceed from the cracks caused by the action of rolling on the ingot and are more dangerous than those seams caused by blow holes in ingots because they all penetrate through the skin of the rail, whereas those resulting from blow holes do not, except in some cases where they are located directly under the outer wall of the ingot.

Blow hole cavities in ingots not containing any foreign matter have been proven by microscopic investigation to weld so perfectly that all traces of same are usually eliminated. We can, therefore, eliminate the seam resulting from blow hole cavities from our consideration of this trouble and confine ourselves to the dangerous seam which penetrates through the skin of the rail. This seam is caused by the action of the blooming rolls on the ingot metal by cracking the sides of the ingot. The structure of the metal in the ingot, as a result of being cast, is of a very coarse crystalline

nature and possessing very little ductility, ruptures when elongated beyond its elastic limit. The work of the blooming mill tends to elongate the ingot very rapidly and before all the four sides of the ingot can be subjected to actual contact with the rolls and receive that amount of work necessary to reduce the coarse crystalline structure and increase the ductility of the metal, the sides, not having had any work, usually rupture. If the ductility of the metal in the walls of the ingot can be increased to any considerable extent before the ingot is bloomed the cause of the dangerous seam in the rail will be largely removed. To accomplish this I propose to subject the ingot to a primary rolling process preferably in front of the soaking pit or heating furnaces. To accomplish this I would put in a small, slow speed-reversing mill, in arrangement the same as an ordinary blooming mill. The ingots, after having been stripped and allowed to reach a satisfactory temperature, would be subjected to the action of the rolls in the mill until the ingot is squared up from top to bottom, and then charged into the soaking pit. The operation of this mill can be regulated so as not to put too severe work on the metal, and by properly designing the rolls a good proportion of the work can be done without unduly elongating the ingot. This form of roll pass is of considerable importance, as it is intended not only to render the metal of the sides of the ingot more ductile, but may have considerable bearing on the pipe in the ingot, which is considered of second importance in causing rail failures.

The primary rolling of the ingot at a time when the ingot may still contain some liquid metal or is still in a plastic condition in the center will, if rolled with the heaviest draft in the direction from bottom to top of ingot, serve to weld the sides of the cavity formed in all ingots as a result of the contraction due to solidification of the metal. After this treatment the ingot should be practically solid from one end to the other and remain so as the temperature of the mass will not be very materially reduced before going to the blooming mill.

It has been found by tests that the seams proceeding from fissures resulting from the heavy reduction in the first few passes through the blooming mill are not welded in later rolling operations and are present

in the finished product. By my method, such seams are eliminated for the reason that the surfaces of the ingot are made tough and dense by reason of the gentler reduction of the first rolling operation, and for the reason that the sides of the ingot are made parallel and the subsequent reduction in the blooming mill is not unequal at different points in the length of the ingot. A result of the elimination of such seams is a rolled product which has a much greater ductility, and its transverse strength is greatly increased. The elimination of the seam, therefore, increases the transverse strength of the rail, which is an object sought. It is obvious that different forms of mechanisms may be employed for carrying out my method. I have, however, shown diagrammatically in the accompanying drawing, an arrangement whereby the method may advantageously be carried out.

In the drawing the figure is a diagrammatic illustration of a rolling mill in which there are shown ingot tracks 10, served by a run-around track 11. The usual soaking pits 12 are provided.

Interposed between the ingot stripping track and the soaking pit is a mill 13, which receives the ingots shortly after they are stripped and by light passes, serves to make uniform the cross section of the ingot at the same time densifying and improving the outer structure thereof and inasmuch as the process is perfectly carried out while the interior of the ingot is still molten, the molten metal will be forced into any pipes which may theretofore have formed. In this preliminary working the ingot is not materially elongated. After leaving the mill 13 the ingots are transferred by the hydraulic pusher 14, to the track 15, which serves the soaking pits. After the ingots are removed from the soaking pits they are delivered at once to the blooming mill 16, from which point the rolling of rails or other shapes.

It will be noted that my novel method has the effect of gently working the sides of the ingot whereby the surfaces thereof are made more dense and homogeneous, these toughened surfaces being thereafter more able to

withstand the heavy reduction in the first pass of the blooming mill. Simultaneously the molten metal contained in the interior of the ingot is pressed into and thereby caused to eliminate any pipes theretofore formed thus making the entire body of the ingot of uniformly homogeneous character and reducing the otherwise crystalline structure of cast bodies.

I claim:

1. A method of treating ingots which consists in subjecting them after stripping from the molds and prior to treatment in a soaking pit, to a rolling action, then reheating the ingots and finally rolling the same into a finished shape, substantially as described.

2. A method of treating ingots which consists in subjecting them after stripping from the molds and prior to reheating in a soaking pit, to a rolling operation whereby the ingot is reduced in cross section and the surfaces thereof rendered more tough, then rebeating the ingot and finally rolling the same into a finished shape, substantially as described.

3. A method of treating ingots which consists in stripping the same from the molds, then slightly reducing the cross sectional area of the ingots by light passes through a rolling mill, whereby the cross section of the ingot is made uniform and the surfaces made more tough and less crystalline, then reheating the ingot, and finally rolling the same into a finished shape, substantially as described.

4. The method of treating ingots, which consists in stripping the same from the mold, then slightly reducing the cross sectional area of the ingot in the rolls of a rolling mill while the interior of the ingot is still in a semi-fluid condition, whereby the cross section of the ingot is made uniform, its surfaces are made tough and less crystalline, then reheating the ingot, and finally rolling the same into the desired form, substantially as described.

HERBERT C. RYDING.

Witnesses:

P. V. KOLB,  
CHAS. F. MURRAY.